

3,503,881  
LIQUID DEVELOPER FOR  
ELECTROPHOTOGRAPHY

Iso Shinohara, Eishun Tsuchida, Toshinao Goto, Zenjiro Okuno, Isao Tashiro, Eiichi Kawamura, and Makoto Nakamura, Tokyo, and Kenkichi Muto, Yokohama, Japan, assignors to Kabushiki Kaisha Ricoh, Tokyo, Japan, a corporation of Japan  
No Drawing. Filed June 20, 1967, Ser. No. 650,565

Int. Cl. G03g 9/06

U.S. Cl. 252—62.1

2 Claims

## ABSTRACT OF THE DISCLOSURE

The invention relates to a liquid developer for use in electrophotography comprising a dispersion into a paraffinic hydrocarbon solvent of a particulated developing agent composed of a reaction product produced by the graft-polymerization to carbon black of acrylate ester having the formula



wherein R<sub>1</sub> is H, CH<sub>3</sub> or C<sub>2</sub>H<sub>5</sub>, and R<sub>2</sub> is C<sub>6</sub>H<sub>13</sub>, C<sub>8</sub>H<sub>17</sub>, C<sub>10</sub>H<sub>21</sub>, C<sub>12</sub>H<sub>25</sub> or C<sub>14</sub>H<sub>29</sub>.

This invention relates to a novel liquid developer to be used for wet development in electrophotography, and further relates to a liquid developer featuring in dispersion a graft-polymer to be used as the particulate developing agent, comprising a pigment and a polarization-control agent having excellent dispersibility in the liquid.

There are two existing methods for development of electrophotography, namely dry method and wet method; the former employs spreading of dry powdered developing agent on the surface of the latent image; the latter employs wet development by the soaking of sensitized material into a liquid developer, in which a developing agent is dispersed in an appropriate solvent. The liquid developer to be used in the wet development method is made from pigment and polarization-control agent by kneading them together into paste, followed by the dispersion of the mixture in an appropriate solvent. Up to the present time, many and various developing agents for use of electrophotography have been proposed; however, commonly used was a rosin, an alkyd resin, and asphalt etc. for dispersing the pigment and for use as a polarization control agent, and a paraffinic hydrocarbon for use as the dispersion medium.

With liquid developers commonly used at present, it is difficult to achieve constant performance as a polarization control agent, because it is derived from naturally occurring materials such as rosin and asphalt. The variations in composition and property of such a natural material would not exist in a manufactured product. In addition, when the developer is used for long term, the dispersibility becomes inferior, and this results in coagulation and precipitation of the particulate developing agent and, therefore causes the development capacity to be lowered, and the image developed to lack sharpness. The deterioration in dispersibility and other defects are believed to result from the fact that the particulate developing agent exists in the liquid in a form to cause the particulate pigment dispersed in the solvent to attract the molecule of polarization control agent in the commencing period of use, so that stabilized dispersion is maintained during this period, but that after repeated use for long term, the dissolved matter separated from

the photoconductive layer of the photosensitive material accumulates, or the molecule of polarization control agent gradually escapes from the particulate pigment owing to the charge of liquid.

The liquid developer of the present invention to be used for electrophotography is a research result achieved after doing wide investigations aimed as improvement in dispersibility and stabilization of particulate developing agent contained in the liquid developer. This does not, at all, use the naturally occurring materials such as rosin and asphalt, and is entirely different from the existing developers, and is an entirely new improved type, having no such defects as mentioned above, and involving the dispersion into the liquid of particulate developing agent obtained by the direct chemical combination of polarization control agent with the pigment. In the liquid developer of the present invention, the monomer of acrylate ester having the following formula is polymerized after kneading with carbon black, initiator of the polymerization reaction, and with benzene, and the particulate developing agent which is formed by the reaction and is in a form having graft-polymerized monomer of acrylate ester onto the particulate carbon, is directly dispersed into paraffinic organic solvent heretofore used for such purposes, to prepare the developer of this invention. In the formula, R<sub>1</sub> is H, CH<sub>3</sub>, or C<sub>2</sub>H<sub>5</sub>; and R<sub>2</sub> is C<sub>6</sub>H<sub>13</sub>, C<sub>8</sub>H<sub>17</sub>, C<sub>10</sub>H<sub>21</sub>, C<sub>12</sub>H<sub>25</sub>, or C<sub>14</sub>H<sub>29</sub>.



As will be exemplified later for purposes of contrasted comparison in the case of polymerization of carbon black with substances other than acrylate ester as presented by the foregoing general formula, for instance, styrene or butyl acrylate etc., the obtained product was, at all, unusable for the purpose as the liquid developer.

The liquid developer to be used in this invention is that illustrated in the foregoing, but the mechanism of the graft-polymerization is not yet clarified at present. Anyhow, this graft polymer of carbon-acrylate ester could become sharply charged developing agent particles by itself when dispersed in ordinary paraffinic solvent, and the dispersibility in the dispersed liquid is quite excellent and displays stabilized development capability even after long term use of the liquid developer. Accordingly, the liquid developer of the present invention could have constant quality which comes from nature of the synthesized raw materials, and furthermore, this does not require various additives as was used in conventional manufacture. However, to obtain further increased sharpness of the image using this developer, the concurrent use of small amount of higher fatty acid or metallic soap is effective.

This invention can be understood better by the detail of the following examples:

## EXAMPLE 1

A 10 gram of lauryl acrylate, 10 gram of carbon black (from Mitsubishi Chemical Company, #44), 0.21 gram of azobisisobutyronitrile (being initiator), and 6.5 gram of benzene were mixed and kneaded, then put into polymerization tube followed by freezing, and degassed under reduced pressure, and was sealed. This was then shaken for 8 hours at 60 deg. C. in the polymerization tank of shaking type. Then, 0.5 gram of the reaction product was put into mortar together with 5 gram of toluene, and after well kneading, this was dispersed into 500 cc. of isoparaffinic hydrocarbon solvent (Isopar H), thus obtaining liquid developer for the use. The particulate developing agent of the liquid developer showed stabil-

ized dispersibility durable for more than 1 month in the liquid. Into this liquid developer, the sensitized material of electrophotography having latent image was immersed, and thus a sharp P/P type image was obtained.

On the other hand, for comparison, another liquid developer was prepared according to the foregoing manner by the use of polymerized product which is form (A) through (D) prescription of the following tabulation, whereas, in the developers thus prepared the particulate developing agent showed decrease in the dispersibility, resulting in coagulation and followed by precipitation.

|        | Carbon<br>Black<br>(g.) | Monomer (g.)           | Benzene<br>(g.) | Azobis<br>isobutyl-<br>onitrile (g.) |
|--------|-------------------------|------------------------|-----------------|--------------------------------------|
| A----- | 10                      | 10 acrylic acid-----   | 23.2            | 0.73                                 |
| B----- | 10                      | 5 acrylic acid-----    | 11.6            | 0.37                                 |
| C----- | 10                      | 10 butyl acrylate----- | 12.2            | 0.38                                 |
| D----- | 10                      | 10 styrene-----        | 15.0            | 0.47                                 |

#### EXAMPLE 2

A 0.5 gram of polymerized product obtained in the former example was kneaded together with 5 grams of toluene, and followed by further addition and kneading with 0.5 gram of 1 percent in toluene solution of aluminum monostearate. This was dispersed into into 500 cc. of isoparaffinic hydrocarbon (Isopar H), thus obtaining liquid developer. Photosensitive material of electrophotography having latent image was immersed into the liquid developer, and P/P type image was obtained which was more sharpened than the former example.

What we claim is:

1. A liquid developer for use in electrophotography comprising a dispersion of particulate developing agent in paraffinic hydrocarbon solvent, said particulate developing agent is composed of reaction product made by graft-polymerization to carbon black with an acrylate ester indicated by the following formula, where;

5 4  
R<sub>1</sub> is H, CH<sub>3</sub> or C<sub>2</sub>H<sub>5</sub>; and R<sub>2</sub> is C<sub>6</sub>H<sub>13</sub>, C<sub>8</sub>H<sub>17</sub>, C<sub>10</sub>H<sub>21</sub>, C<sub>12</sub>H<sub>25</sub>, or C<sub>14</sub>H<sub>29</sub>.



10 10  
2. A liquid developer for use in electrophotography comprising a dispersion of particulate developing agent and a small amount of a metallic soap, into paraffinic hydrocarbon solvent, said particulate developing agent composed of reaction product made by graft-polymerization to carbon black with an acrylate ester indicated by the following formula, where; R<sub>1</sub> is H, CH<sub>3</sub> or C<sub>2</sub>H<sub>5</sub>; and R<sub>2</sub> is C<sub>6</sub>H<sub>13</sub>, C<sub>8</sub>H<sub>17</sub>, C<sub>10</sub>H<sub>21</sub>, C<sub>12</sub>H<sub>25</sub>, or C<sub>14</sub>H<sub>29</sub>.



#### References Cited

##### UNITED STATES PATENTS

- 3,272,772 9/1966 Russell ----- 106—3.8  
3,385,808 5/1968 Bonin et al. ----- 106—3.8

##### FOREIGN PATENTS

- 859,292 1/1961 Great Britain.  
869,391 5/1961 Great Britain.

30 30 GEORGE F. LESMES, Primary Examiner

J. P. BRAMMER, Assistant Examiner

U.S. CL. X.R.

35 106—308; 117—37; 260—41

UNITED STATES PATENT OFFICE  
CERTIFICATE OF CORRECTION

Patent No. 3503881 Dated March 31, 1970

Inventor(s) Isao Shinohara, Eishun Tsuchida, Toshinao Goto,  
Zenjiro Okuno, Isao Tashiro, Eiichi Kawamura,

Makoto Nakamura, and Kenkichi Muto

It is certified that error appears in the above-identified patent  
and that said Letters Patent are hereby corrected as shown below:

Column 4, line 14, after "CH<sub>3</sub>" insert --,--; line 14,  
the formula reading "C<sub>6</sub>H<sub>17</sub>" should read -- C<sub>8</sub>H<sub>17</sub> --.

SIGNED AND  
SEALED

JUL 28 1970

(SEAL)

Attest:

Edward M. Fletcher, Jr.

Attesting Officer

WILLIAM E. SCHUYLER, JR.  
Commissioner of Patents